

## UNITED STATES PATENT OFFICE

2,229,946

COMPOSITION FOR MOLDS FOR METAL  
CASTING

George Clyde Van Allen, Maplewood, N. J., assignor to Baker &amp; Company, Inc., Newark, N. J., a corporation of New Jersey

No Drawing. Application February 8, 1938,  
Serial No. 189,319

## 1 Claim. (Cl. 22—188)

This invention relates to investment compositions for the making of refractory molds for use in casting metals, alloys and other suitable casting materials. The composition is particularly intended for use in molds for casting dental inlays, dentures and the like, although the composition is equally adaptable for use in molds for casting articles of jewelry and other objects.

Known investment compositions of this general character generally comprise a ground siliceous refractory base such as silica in its various forms, and a binder such as a gypsum product, for example calcined gypsum or plaster of Paris. Other ingredients or agents for the purpose of accelerating or retarding hardening, setting or expansion of the composition, or to modify the plasticity of the composition to facilitate mixing and shaping thereof, are also frequently included in such investment compositions.

The customary procedure in making molds of such compositions and casting articles therein, consists in shaping a preliminary wax model or pattern of the object to be cast, for example a dental inlay, mixing the investment composition with a suitable liquid, for example water, constructing the mold around the pattern, allowing the mold to set, heating the set mold slowly to drive out the moisture and melt and burn out the wax pattern, and continuing heating until the mold is sufficiently hot to compensate for the shrinkage of the cast material as well as to eliminate all wax and residue from same so as to leave a cavity corresponding in shape and size to the model, then pouring the molten casting material, for example gold, into the heated mold cavity and allowing the casting to cool.

Generally the molds are heated to a temperature of from 900° F. to 1500° F. before the casting is formed, which causes the mold to expand, and the casting material after having been put in the mold cavity usually shrinks during cooling. Therefore, in order to obtain a casting which shall conform exactly in size and shape to the model, the expansion of the mold must correspond as exactly as possible to the shrinkage of the casting material. Generally this expansion is slightly above 1%, for example in the case of casting gold, about 1.25%.

While such investment compositions compris-

ing only a ground siliceous refractory material, such as silica, and a binder such as plaster of Paris, have the property of expansion under heat, the degree of expansion is not sufficient to compensate entirely for the shrinkage of the casting material. As an example, we find that a composition comprising seventy percent (70%) of silica and thirty percent (30%) of plaster of Paris has a maximum expansion of about eighty-six hundredths of one percent (0.860%) at a temperature of fifteen hundred (1500) degrees F. which is insufficient to compensate for the average shrinkage of the casting material of from one (1) to one and one-quarter (1 1/4) percent. A decrease of the silica content and a corresponding increase in the plaster of Paris content will result in a considerably smaller expansion of the composition during heating.

To increase the expansion of the investment composition, it is customary practice to include therein so-called expansion agents or expansion promoters, such as oxalic acid or citric acid or sodium chloride.

Prime object of my invention is to provide an investment composition which shall include a new and improved combination of constituents or ingredients one or more of which shall make it possible to obtain exactly the desired degree of expansion of the composition during heating thereof.

I have discovered that the desired expansion characteristics of investment compositions can be obtained, and the degree of expansion of such compositions can be increased substantially, by incorporating in such compositions small quantities of one or more substances of the group consisting of ammonium chloride, aluminum chloride, ammonium bromide, and sodium nitrate.

As examples, sodium nitrate and ammonium bromide together may be added as expansion agents to the other constituents of the composition, or ammonium chloride and aluminum chloride together may be used as expansion agents; and if desired all four of my enumerated expansion agents may be used together.

The addition of one or more of my expansion agents to an investment composition remarkably improves the expansion characteristics of the composition and strikingly increases the degree of expansion. Whereas, as above pointed out a

composition with a base of 70% silica and 30% of plaster of Paris has a maximum expansion of 0.860% at about 1500° F., the substitution of 1% of my expansion agents for an equal amount of the silica or plaster of Paris produces at the same temperature the following maximum expansions.

|    | Expansion agent        | Percent expansion |
|----|------------------------|-------------------|
| 10 | Sodium nitrate.....    | 1.035             |
|    | Ammonium chloride..... | 1.040             |
|    | Aluminum chloride..... | 1.180             |
|    | Ammonium bromide.....  | 1.205             |

- 15 The proportions of my expansion agents in the investment composition may be varied from one-quarter of one percent (0.25%) to about three percent (3%) by weight. The preferred range lies between three-quarters of one percent (0.75%) to two percent (2%), although the most satisfactory proportions with the proportions of the other ingredients now used, are from one percent (1%) to one and three-tenths percent (1.30%).
- 20 The proportion of the refractory base or filler, for example silica, may be varied widely, for ex-

ample from forty percent (40%) to eighty-five percent (85%), while the proportion of the binder, for example calcined gypsum or Portland cement, may also vary within a wide range, for example from fifteen percent (15%) to sixty percent (60%). Preferably, in all cases, the materials comprise particles of different sizes.

5 Each of my expansion agents may be used alone, or in combination with others of my expansion agents, or in combination with other expansion agents or promoters.

Also, my expansion agents may be utilized in investment compositions with ingredients or agents for accelerating or retarding setting or hardening of the compositions, or for modifying 15 plasticity or other qualities or characteristics of the compositions.

Having thus described my invention, what I claim is:

An investment composition comprising from 20 forty percent (40%) to eighty percent (80%) of silica, from fifteen percent (15%) to sixty percent (60%) of plaster of Paris, and from one-quarter (0.25%) to three percent (3%) of ammonium bromide.

25 G. CLYDE VAN ALLEN.